

## UNITED STATES PATENT OFFICE

2,096,705

PROCESS OF SOFTENING FIBERS AND  
PRODUCTS THEREOF

Howard Heckethorn, Oswego, N. Y., assignor of  
one-third to Warren K. Cooley, Silver Spring,  
Md., and one-third to Edward M. Schenke,  
Chevy Chase, Md.

No Drawing. Application October 28, 1930,  
Serial No. 491,810

30 Claims. (Cl. 28—59)

This invention relates to processes of softening fiber and products thereof; and it comprises a method of temporarily softening and lubricating rayon, acetate silk, natural silk and other fibers, threads or filaments wherein fiber is treated with a substantially homogeneous mobile and thinly liquid composition containing an anhydrous solvent, usually a close boiling naphtha and a soap of an organic base, usually a soap of an ethanolamine; and the soap being one which will blend and go into homogeneous mixture with said solvent; all as more fully hereinafter set forth and as claimed.

In working fiber and thread, by spinning, throwing, twisting, winding, knitting, braiding, weaving and like operations, there is considerable expenditure of energy in and on the fiber and it is customary to use a softening agent to reduce stiffness, aid flexure and facilitate the relative movement of the sub-fibers. For an ideal softener the requirements are exacting and, to some extent, conflicting. Chief among these requirements is that the softening agent shall be easily and uniformly applied in the exact small quantities required prior to the working operation and that it shall be susceptible of quick and complete removal afterwards. None of the usual softening agents meets both these requirements to an extent desirable; and particularly with softening agents used for rayon and other forms of synthetic fibers or filaments which have a quite different physical character from the older fibers. Hydrocarbon oils of the character of the wool oils are easily and uniformly applied although not readily in exact small quantity but they offer difficulty in complete removal and their removal requires considerable care and precaution. So far as ease of removal is concerned the ordinary soda and potash soaps are good and they are desirable softening agents in the fiber. But to apply them in small quantity and secure even and uniform penetration of the fiber is not easy although it may be done as hereinafter pointed out. Emulsions of oil in various vehicles are often used but the emulsion must be very fine to prevent a filtering action by the fiber.

In the present invention these objections are overcome by the use of a soap, or other softening agent, dissolved in a suitable solvent to give a mobile penetrating solution. The necessary quantity of softening agent is applied to the fiber in the solution and then the solvent evaporated off, leaving the softening agent in place. For my purposes I frequently use soaps. Advantageously, the soap is made with an organic base soluble in hy-

drocarbons as this permits the use of a simple hydrocarbon solvent. Ordinary soda and potash soap may however be used with hydrocarbons if there be included a co-solvent enabling the production of a true solution; a solvent miscible with the hydrocarbon and capable of dissolving the soap.

Ordinary soda and potash soaps are not soluble in the usual hydrocarbons to form any true solution. The true solubility of a dry soap, soda or potash soap, as distinguished from a dispersion, in petroleum oils is probably less than 0.5 per cent by weight. On the other hand the substituted ammonias carrying hydrocarbon radicals are soluble in hydrocarbons to an extent dependent upon the degree of substitution; and their soaps with fatty acids are also soluble. Various soaps of organic bases are useful and among them are the soaps formed by certain bases known as ethanolamines. The ethanolamines are formed by the reacting ammonia with ethylene oxide. Similar bases are formed by propylene oxide and these are even more advantageous for the present purposes although commercially not so available. Monoethanolamine, diethanolamine and triethanolamine are all applicable for the present purposes as is the commercial mixture of the three bases sold as "triethanolamine". As the fatty acid there may be used commercial oleic acid or any other convenient soap making acid. The free fatty acids from cocoanut oil are commercially available, are relatively cheap and are quite advantageous for the present purposes. These fatty acids, or any other fatty acid, may be directly saponified by triethanolamine.

One advantage of the ethanolamine soaps in hydrocarbon solution for the present purposes is their relative tolerance for moisture. A solution of the soap in naphtha tolerates the presence of a substantial amount of moisture without losing homogeneity.

In softening and lubricating rayon fiber as a rule the amount of soap required in the fiber is not more than about 4 to 6 parts by weight per 100 parts of fiber; and it is difficult, for reasons stated ante to get this small amount into and through the fiber uniformly. I therefore use a solution of the ethanolamine soap in a hydrocarbon solvent to produce impregnation with enough solvent to produce a mobile or thinly liquid composition. After impregnation the solvent is removed by evaporation, as by exposure to air. For this purpose any hydrocarbon solvent boiling with a fairly definite end point and not too volatile may be used. A solvent containing much

"heavy ends" is objectionable since it leaves oil in the fiber which must be subsequently removed. The solvents should also be free, or reasonably free, of unsaturated bodies since these may lead 5 to oxidation and tendering of the fiber. A good solvent for the present purposes is a material used by dry cleaners and known as "Stoddard Solvent"; a close boiling naphtha fraction having an over point of 300° F. and an end point of 10 410° F. This Stoddard solvent is sold under specifications requiring that the content of unsaturates shall be less than 5 per cent. However, any hydrocarbon oil, such as commercial benzol, toluene or naphtha fractions may be used; it being 15 merely necessary that the flash point of the liquid used be high to preclude fire danger and that the end point be fairly definite to avoid contaminating the fiber with heavy oils.

For the present purposes a solution of ethanolamine soaps in "Stoddard Solvent" carrying 20 to 50 per cent of such soap may be used. Something depends on the permeability of the fiber and the amount of softener wanted in it. Solutions of these soaps, containing between 20 to 25 30 per cent of soap are efficient. If the particular hydrocarbon used as a solvent or extending agent be too volatile it is often desirable to add some carbon tetrachlorid to raise the flash point. If there is much moisture to be dealt with, it is 30 sometimes desirable to add some proportion of an ordinary solvent miscible with both water and hydrocarbons, such as butyl alcohol, cyclohexanol, etc. The amount of such an addition, however, is usually small; it being regarded as desirable 35 that the softening and lubricating agent for the present purposes consist mainly of the organic base soap and a dry hydrocarbon extender or solvent.

In the performance of the present process, 40 the starting materials in any suitable form, such as threads, yarns, filaments or the like, are impregnated with a mobile solution of the softening and lubricating agent in a volatile hydrocarbon solvent of the character stated. The volatile solvent 45 is then evaporated off and, if desired, recovered. The impregnated materials thus obtained are subjected to any of the usual operations, such as spinning, weaving, twisting or the like, to form the desired textile articles. After 50 such operations are completed, the textile products are worked in water or dilute soap solutions, to wash out and remove the softening and lubricating agent, and the washed products rinsed in clear water and then dried.

55 While I have disclosed my invention more particularly in its use with a hydrocarbon solution of a soap having an organic base and while I regard this as the most advantageous embodiment of my invention, the principles of my invention 60 can be used with other compositions. I can for instance dissolve 20 or 30 per cent of potash soap in a compound solvent consisting of "Stoddard Solvent" admixed with butanol or cyclohexanol or any other moderately high boiling 65 organic solvent which will act as a co-solvent for soap and for hydrocarbon. This solution of soap is applied to the fiber or thread as before to secure impregnation with the necessary exact 70 small quantity of soap, the solvent is removed by evaporation, the fiber worked in such ways as may be necessary and the impregnating soap removed by washing as before.

The butanol or cyclohexanol has another function in addition to acting as a co-solvent, since

it takes care of the water of condition taken up from the fiber by the mixed solvent.

My dry solvent-soap solution may be used to impregnate all types of textile materials with a softening and lubricating agent. Animal, vegetable or synthetic fibers, filaments, or threads may be treated. Typical examples of animal fibers are natural or boiled-off silk, tussah silks, wool, hairs, etc. Of vegetable fibers there may be mentioned cotton, mercerized cotton, linen, ramie, 10 hemp, jute, manila, kapok and the like. All synthetic fibers, such as viscose, cuprammonium, nitrocellulose and cellulose acetate silks, may be advantageously treated with my compositions.

The impregnated textile materials can then be 15 worked in any desired manner to fabricate the material into various products. They may be subjected to any of the usual manipulations such as spinning, throwing, twisting, winding, knitting, braiding or weaving. The desired manipulations 20 may be performed with great facility and speed without any of the danger of damaging the material usually attending such manipulations of these materials.

After performing the desired working the softening and lubricating agent, may be, as stated, easily and quickly removed by simple washing; complete removal is readily effected. This may be done in various ways. The material may be worked in hot water. About one-half hour with 30 water heated to between 100° F. to 140° F. is sufficient in most cases. Then it is rinsed in clear water, advantageously at about 100° F. Instead of washing with hot water, a dilute soap solution at a somewhat lower temperature may be 35 used. With a dilute soap solution a subsequent rinsing with clear water is also used. If desired varying amounts of alkaline materials such as trisodium phosphate or soda ash, may be added to the dilute soap solution. Or these dilute alkali 40 solutions may be used alone for the washing. However, the use of dilute alkaline solutions or their addition to dilute soap solutions is only recommended, when it is desired there be simultaneous cleansing to remove foreign bodies originally present in the textile material or which may have been picked up during the working or manipulation. When, however, it is necessary to remove only the softening and lubricating agent from the impregnated material, alkalies etc., are 45 not needed.

Frequently, after working, it is desired to dye the textile material. With softening and lubricating agents of the ethanolamine-fatty acid soap type, it is not ordinarily necessary to effect removal before dyeing the material. If the dye bath to be used is either neutral or alkaline, the impregnated material may be directly entered into the dye bath. Dyeing and the removal of the softening or lubricating agent are simultaneously effected. When the material is worked in the dye bath in the usual manner, the softening and lubricating agent is washed out. With ethanolamine soap, most dye baths are unaffected. This type of soap has no "salting out" effect, like 65 that of ordinary soaps. In fact, it aids in the penetration of the dye into the material. After dyeing the material is rinsed in the customary manner.

The following examples serve to illustrate certain embodiments of my invention; but they in no way limit the broad scope of my invention as set forth ante. The parts are given as parts by weight.

Examples 1 to 3 set forth typical compositions

which contain an organic base-soap dissolved in an organic hydrocarbon solvent.

*Example 1*

5 235 parts of cocoanut oil acids are saponified with 120 parts commercial triethanolamine to obtain a softening and lubricating agent. The soap thus obtained is mixed with and dissolved in a hydrocarbon solvent; which may be a mixture of 10 1345 parts of "Stoddard Solvent" and 36 parts of butyl "cellosolve" or hexalin. The composition thus formed may be used to impregnate all types of textile materials. Various other fatty acids may be used in lieu of the fatty acids of cocoanut 15 oil. Also the type and proportion of the hydrocarbon solvent may be varied within wide limits.

*Example 2*

20 220 parts of commercial oleic acid are saponified with 100 parts of commercial triethanolamine. The soap thus obtained is then dissolved in an oily solvent comprising 1,000 parts of Stoddard Solvent, 400 parts of carbon tetrachlorid and 100 parts of colorless high boiling mineral oil. 25 The mineral oil in the small amount stated is easily removed in washing out the soap. This oil is itself a softening and lubricating agent. This composition not only contains an organic base-soap as a softening and lubricating agent but also an added softening agent, namely, colorless mineral oil. The carbon tetrachlorid also adds certain desired properties to the composition. The stated composition may also be varied within wide limits and in place of the mineral 30 oil, as an added softening and lubricating agent, other softening and lubricating agents may be substituted in lieu thereof to produce an impregnating composition containing two or more softening and lubricating agents.

40 In the above examples the hydrocarbon solvent has Stoddard Solvent as a basis, but various other organic solvents commonly known as dry solvents in dry cleaning, may be used in lieu thereof either alone or in various mixtures. The following example is typical of such modifications.

*Example 3*

220 parts of commercial oleic acid are saponified with 100 parts of triethanolamine. The resulting soap is dissolved in a dry solvent comprising 100 parts of carbon tetrachlorid and 40 parts of hexalin. The hexalin imparts certain advantageous properties and functions also as a co-solvent, that is a blending or carrying agent, assisting in blending the softening agent with tetrachlorid. The homogeneous impregnating compositions obtained are, or behave, as true solutions. In place of the hexalin various other co-solvents, for instance, butanol, amyl alcohol, "cellosolve" or butyl "cellosolve" may be used. Chemically "cellosolve" is mono-ethyl ether of ethylene glycol. Also certain amounts of free fatty acids exercise like action. Free fatty acids may be added to the impregnating compositions or the fatty acids used may be only partially saponified, leaving an excess of free fatty acids.

70 The above examples illustrate the use of an organic base-soap type of softening and lubricating agent. However as stated by a variation in solvents, there may be used as a softening and lubricating agent soaps obtained by combining fatty acids with alkalies, namely, caustic soda or potash. The following example illustrates this 75 modification.

*Example 4*

100 parts of commercial oleic acid are saponified with alcoholic caustic potash; using a mixture of 19 parts of caustic potash with 30 parts of methyl alcohol. The reaction mixture thus obtained is mixed with a hydrocarbon solvent comprising 450 parts of Stoddard Solvent and 35 parts of hexalin. A homogeneous impregnating composition is obtained, which may be effectively used in our process. In making impregnating compositions of this type it is advisable to have a substantial amount of a co-solvent, that is, blending or carrying agent, such as the hexalin and alcohol in the above composition.

The above examples are merely typical embodiments and compositions under the present invention may be varied over a wide range to suit them for a particular application or use. All these compositions comprise essentially an organic or hydrocarbon solvent of the type known as dry solvents with a softening and lubricating agent dissolved therein. Various hydrocarbon and other organic solvents may be used in making these compositions. Stoddard Solvent is advantageous but other organic solvents such as carbon tetrachlorid, ethylene dichlorid, chloroform, trichlorethylene, tetrachlorethane, isopropanol or other alcohols, or any desired mixture or mixtures of these solvents may be used. The softening and lubricating agent may be advantageously, organic base-fatty acid soap-like products for the stated reasons.

Where additional softening agents are used they may be added, the solvent employed being one which will dissolve mineral oil, vegetable oil, animal oil, sulfonated oils, etc. At times it is desirable to use a modicum of such an oil as olive oil, castor oil, rape seed oil, soy bean, cotton-seed oil etc. neatfoot oil, olein. Turkey red oil may be incorporated.

Sometimes it is desired to dye textile materials prior to fabricating them into textile products. With my compositions it is possible to simultaneously impregnate and dye the textile material. For this purpose suitable dyes may be incorporated with my impregnating compositions. In certain textile operations it is desired to easily identify certain materials during the processing; to this end they are dyed. In such instances, the dyes may be such that they may be stripped from the fiber when it is washed to remove the softening and lubricating agent; the dyeing being merely for identification during the process.

Liquid compositions under the present invention may be applied to thread or fabric to secure impregnation in any of the usual ways; as by dipping or immersing, spraying, transferring by rolls, etc. Capillary action may be relied upon; a wick action so to speak. In impregnation the material to be treated may be handled in any of the usual ways, as on bobbins, skeins, cones, etc. In removing the solvent this may be done by simple exposure to air which may be at atmospheric temperature, or may be at higher temperature, or special means employing a current of air may be used to remove and recover the solvent. In removing the solvent sufficient time should always be allowed to permit diffusion of solvent from the textile and equalization of the softening agent in the thread, etc.

In addition to the stated use of compositions under the present invention in affording lubrication and softening, they are also applicable to finishing materials to enhance the feel and luster.

of goods. In so doing somewhat more dilute solutions are more desirable than those hereinbefore recited.

Where the word "silk" is used in the appended 5 claims as specifying the particular type of fiber, it is used in its broad sense and includes, in addition to natural silk, the various types of artificial fibers which are generally considered as artificial silk.

10 What I claim is:

1. In a process for temporarily softening and lubricating textile fibers which are to be used in textile operations, the step which comprises impregnating such fibers with a liquid solution capable of rendering said fibers soft and pliable and readily workable on textile machines, said solution comprising a water-soluble soap capable of acting as a softening and lubricating agent and an organic solvent therefor in which the textile 15 fibers are insoluble.

2. In a process for temporarily softening and lubricating textile fibers which are to be used in textile operations, the step which comprises impregnating such fibers with a liquid solution capable of rendering said fibers soft and pliable and readily workable on textile machines, said solution comprising a water-soluble soap capable of acting as a softening and lubricating agent and a volatile hydrocarbon solvent therefor.

3. In a process for temporarily softening and lubricating textile fibers which are to be used in textile operations, the step which comprises impregnating such fibers with a liquid solution capable of rendering said fibers soft and pliable and readily workable on textile machines, said solution comprising naphtha and a water-soluble soap capable of acting as a softening and lubricating agent dissolved therein.

4. In a process for temporarily softening and lubricating textile fibers which are to be used in textile operations, the step which comprises impregnating such fibers with a liquid solution capable of rendering said fibers soft and pliable and readily workable on textile machines, said solution comprising an organic solvent in which the textile fibers are insoluble, a softening and lubricating agent normally insoluble therein and a co-solvent for the organic solvent and the softening and lubricating agent.

5. In a process for temporarily softening and lubricating textile fibers which are to be used in textile operations, the step which comprises impregnating such fibers with a liquid solution capable of rendering said fibers soft and pliable and readily workable on textile machines, said solution comprising an organic solvent in which the fibers are insoluble, a water-soluble soap capable of acting as a softening and lubricating agent which is normally insoluble in said organic solvent, and a co-solvent for the organic solvent and soap.

6. In a process for temporarily softening and lubricating textile fibers which are to be used in textile operations, the step which comprises impregnating such fibers with a liquid solution capable of rendering said fibers soft and pliable and readily workable on textile machines, said solution comprising a volatile hydrocarbon solvent, a water-soluble soap capable of acting as a softening and lubricating agent which is normally insoluble therein and a co-solvent for the volatile hydrocarbon solvent and the soap.

7. In a process for temporarily softening and lubricating textile fibers which are to be used in textile operations, the step which comprises im-

pregnating such fibers with a liquid solution capable of rendering said fibers soft and pliable and readily workable on textile machines, said solution comprising naphtha, a water-soluble soap normally insoluble therein and a co-solvent for the naphtha and soap.

8. In a process for temporarily softening and lubricating textile fibers which are to be used in textile operations, the step which comprises impregnating such fibers with a liquid solution capable of rendering said fibers soft and pliable and readily workable on textile machines, said solution comprising an organic solvent in which the textile fibers are insoluble, a softening and lubricating agent normally insoluble in said organic solvent and a co-solvent for the organic solvent and the softening and lubricating agent from the class consisting of alcohol, amyl alcohol, cyclo-hexanol, butanol and monoethylether of ethylene glycol.

9. In a process for temporarily softening and lubricating textile fibers which are to be used in textile operations, the step which comprises impregnating such fibers with a liquid solution capable of rendering said fibers soft and pliable and readily workable on textile machines, said solution comprising an oil, a soap capable of acting as a softening and lubricating agent and an organic solvent for the oil and soap in which the fibers are insoluble.

10. In a process for temporarily softening and lubricating textile fibers which are to be used in textile operations, the step which comprises impregnating such fibers with a liquid solution capable of rendering said fibers soft and pliable and readily workable on textile machines, said solution comprising a water-soluble soap capable of acting as a softening and lubricating agent and an organic solvent therefor in which the textile fibers are insoluble, subsequently working the fiber, and thereafter washing said impregnated fiber to remove the soap.

11. In a process for temporarily softening and lubricating textile fibers which are to be used in textile operations, the step which comprises impregnating such fibers with a liquid solution capable of rendering said fibers soft and pliable and readily workable on textile machines, said solution comprising an organic solvent in which the textile fibers are insoluble, a water-soluble soap capable of acting as a softening agent which is normally insoluble in said organic solvent and a co-solvent for the organic solvent and soap, removing the solvent and the co-solvent, subsequently working the fiber, and thereafter washing said impregnated fiber to remove the soap.

12. In a process for temporarily softening and lubricating silk which is to be used in a textile operation, the step which comprises impregnating the silk with a liquid solution capable of rendering the silk soft and pliable and readily workable on textile machines, said solution comprising a water-soluble soap capable of acting as a softening and lubricating agent and an organic solvent for the soap in which the silk is insoluble.

13. As a new composition for softening and lubricating textile fibers which are to be used in textile operations, a liquid solution comprising an organic solvent in which the textile fibers are insoluble and a water-soluble soap capable of acting as a softening and lubricating agent dissolved in the solvent, said solution being capable of readily penetrating a textile fiber by gravity and rendering the same soft and pliable and readily workable on textile machines.

14. As a new composition for softening and

5 lubricating textile fibers which are to be used in textile operations, a liquid solution comprising a volatile hydrocarbon solvent and a water-soluble soap capable of acting as a softening and lubricating agent dissolved therein, said solution being capable of readily penetrating a textile fiber by gravity and rendering the same soft and pliable and readily workable on textile machines.

10 15. As a new composition for softening and lubricating textile fibers which are to be used in textile operations, a liquid solution comprising naphtha and a water-soluble soap capable of acting as a softening and lubricating agent dissolved in the naphtha, said solution being capable of readily penetrating a textile fiber by gravity and rendering the same soft and pliable and readily workable on textile machines.

15 20 25 30 35 40 45 50 55 60 65 70 75 16. As a new composition for softening and lubricating textile fibers which are to be used in textile operations, a liquid solution comprising an organic solvent in which the textile fibers are insoluble, at least one softening and lubricating agent normally insoluble in said organic solvent and a co-solvent for the organic solvent and the softening and lubricating agent, said solution being capable of readily penetrating a textile fiber by gravity and rendering the same soft and pliable and readily workable on textile machines.

17. As a new composition for softening and lubricating textile fibers which are to be used in textile operations, a liquid solution comprising an organic solvent in which textile fibers are insoluble, a water-soluble soap capable of acting as a softening and lubricating agent which is normally insoluble in said organic solvent, and a co-solvent for the organic solvent and the soap, said solution being capable of readily penetrating a textile fiber by gravity and rendering the same soft and pliable and readily workable on textile machines.

18. As a new composition for softening and lubricating textile fibers which are to be used in textile operations, a liquid solution comprising a volatile hydrocarbon solvent, a water-soluble soap capable of acting as a softening and lubricating agent which is normally insoluble in said volatile hydrocarbon, and a co-solvent for the volatile hydrocarbon and the soap, said solution being capable of readily penetrating a textile fiber by gravity and rendering the same soft and pliable and readily workable on textile machines.

19. As a new composition for softening and lubricating textile fibers which are to be used in textile operations, a liquid solution comprising naphtha, a water-soluble soap capable of acting as a softening and lubricating agent which is normally insoluble in said naphtha, and a co-solvent for the naphtha and soap, said solution being capable of readily penetrating a textile fiber by gravity and rendering the same soft and pliable and readily workable on textile machines.

20. As a new composition for softening and lubricating textile fibers which are to be used in textile operations, a liquid solution comprising an organic solvent in which textile fibers are insoluble and a water-soluble soap capable of acting as a softening and lubricating agent dissolved in the solvent, the softener and lubricant comprising at least 10% of the solution, said solution being capable of readily penetrating a textile fiber by gravity and rendering the same soft and pliable and readily workable on textile machines.

21. As a new composition for softening and lubricating textile fibers which are to be used in textile operations, a liquid solution comprising a volatile hydrocarbon solvent and a water-soluble

5 soap capable of acting as a softening and lubricating agent dissolved therein, the softener and lubricant comprising at least 10% of the solution, said solution being capable of readily penetrating a textile fiber by gravity and rendering the same soft and pliable and readily workable on textile machines.

10 15 20 25 30 35 40 45 50 55 60 65 70 75 22. As a new composition for softening and lubricating textile fibers which are to be used in textile operations, a liquid solution comprising naphtha and a water-soluble soap capable of acting as a softening and lubricating agent dissolved in the naphtha, the softener and lubricant comprising at least 10% of the solution, said solution being capable of readily penetrating a textile fiber by gravity and rendering the same soft and pliable and readily workable on textile machines.

23. As a new composition for softening and lubricating textile fibers which are to be used in textile operations, a liquid solution comprising an oil, a water-soluble soap capable of acting as a softening and lubricating agent and an organic solvent for the oil and soap in which the fibers are insoluble, said solution being capable of readily penetrating a textile fiber by gravity and rendering the same soft and pliable and readily workable on textile machines.

28. As a new composition for softening and lubricating textile fibers which are to be used in textile operations, a liquid solution comprising an organic solvent in which textile fibers are insoluble, and an ethanol amine soap dissolved in the solvent, said solution being capable of readily penetrating a textile fiber by gravity and rendering the same soft and pliable and readily workable on textile machines.

33. As a new composition for softening and lubricating textile fibers which are to be used in textile operations, a liquid solution comprising an organic solvent in which the textile fibers are insoluble, a softening and lubricating agent other than a soap, and an ethanol amine soap, the softening and lubricating agent and the soap being dissolved in the solvent and the solution being capable of readily penetrating a textile fiber by gravity and rendering the same soft and pliable and readily workable on textile machines.

38. As a new composition for softening and lubricating textile fibers which are to be used in textile operations, a liquid solution comprising an organic solvent in which the textile fibers are insoluble, a softening and lubricating agent normally insoluble in said organic solvent, and a co-solvent for the organic solvent and the softening and lubricating agent from the class consisting of alcohol, amyl alcohol, cyclo-hexanol, butanol and monoethylether of ethylene glycol, said solution being capable of readily penetrating the textile fibers by gravity and rendering the same soft and pliable and readily workable on textile machines.

43. In a process for temporarily softening and lubricating synthetic textile fibers which are to be used in textile operations, the step which comprises impregnating the fibers with a liquid solution capable of rendering said fibers soft and pliable and readily workable on textile machines, said solution comprising a water-soluble soap capable of acting as a softening and lubricating agent and an organic solvent for the soap in which the fibers are insoluble.

48. In a process for temporarily softening and lubricating textile fibers composed of cellulose acetate which are to be used in textile opera-

- tions, the step which comprises impregnating the fibers with a liquid solution capable of rendering said fibers soft and pliable and readily workable on textile machines, said solution comprising a water-soluble soap capable of acting as a softening and lubricating agent and an organic solvent for the soap in which the fibers are insoluble.
29. In a process for temporarily softening and lubricating synthetic textile fibers which are to be used in textile operations, the step which comprises impregnating the fibers with a liquid solution capable of rendering said fibers soft and pliable and readily workable on textile machines, said solution comprising an organic solvent in which the synthetic fibers are insoluble, a water-soluble soap capable of acting as a softening
- 10
- 15

agent which is normally insoluble in said organic solvent and a co-solvent for the organic solvent and the soap.

30. In a process for temporarily softening and lubricating textile fibers composed of cellulose acetate which are to be used in textile operations, the step which comprises impregnating the fibers with a liquid solution capable of rendering said fibers soft and pliable and readily workable on textile machines, said solution comprising an organic solvent in which the fibers are insoluble, a water-soluble soap capable of acting as a softening agent which is normally insoluble in said organic solvent and a co-solvent for the organic solvent and the soap.

HOWARD HECKETHORN.